

D. J. O'HARRA & C. B. THOMPSON.  
FURNACE FOR ROASTING ORES.

No. 67,445.

Patented Aug. 6, 1867.



Witnesses  
Amahon  
Thos J. Chamberlain

Inventor  
David Jones, Almaria  
Clark Brown Thompson  
By their Atty J. Dennis Jr

# United States Patent Office.

DAVID JONES O'HARRA AND CLARK BROWN THOMPSON, OF EMPIRE CITY,  
NEVADA.

*Letters Patent No. 67,445, dated August 6, 1867.*

## IMPROVED FURNACE FOR ROASTING ORES.

The Schedule referred to in these Letters Patent and making part of the same.

TO ALL WHOM IT MAY CONCERN:

Be it known that we DAVID J. O'HARRA and CLARK B. THOMPSON, of Empire City, Ormsby county, State of Nevada, have invented certain new and useful "Improvements in Furnaces" for Desulphurizing and Chloridizing Ores; and we do hereby declare the following description and accompanying drawings are sufficient to enable any person skilled in the art or science to which it most nearly appertains to make and use our said invention without further invention or experiment.

The nature of our invention relates to the employment of a longitudinal furnace, more especially adapted to the roasting of ores, having a flat sole and roof in order to confine the heat to the bottom and surface of the ore, and heat it up gradually, the fire being placed at intervals along the said furnace, and the ore stirred at intervals by hoes attached to an endless chain passing through it. The furnace being open at both ends the hoes receive the ore at one end and discharge it at the other roasted. Referring to the drawings—

Figure 1 represents a side elevation of our furnace.

Figure 2, a plan.

Figure 3, an end view.

Figures 4 and 5, plan of hoes or conveyers.

We construct our furnace of the usual materials and of different dimensions. We think about eighty feet long and forty-one feet wide the most suitable size.

The hearth A is a perfect plane as well as the flat roof B. At each end of the furnace we attach a grooved pulley, C and C'. Around these pulleys passes an endless chain, D, passing completely through the furnace. Conveyers E and E' are attached to this chain at equal distances, and are constructed in the form of a circular iron frame divided into two semicircles along a line perpendicular to its line of motion, and hinged with hook and eye to allow it to double together in passing over the pulleys C C'. On the bottom of these conveyors we place four hoes a a a a at an angle of about forty-five degrees with the axis of the furnace, while the centre hoe is composed of two hoes inclined towards each other, and firmly attached together along their forward vertical edge, forming an instrument resembling a double mould-board plough. This hoe ploughs through the ore along the centre of the hearth, throwing it in either direction and leaving a furrow behind it. The hoes on the opposite edge of the circular plate, however, following the leading hoe, and having their faces inclined in the opposite direction, throw the ore back and fill up the furrow again. All the hoes attached to the circular plate are arranged and inclined, as shown in the drawings, with special reference to producing this effect upon the ores, alternately ploughing them in one direction and then in the other, so as to produce a thorough agitation of the contents of the ore-chamber. The circular plates or conveyers are made of sufficient size to extend across the entire width of the hearth, and are attached in a suitable manner to the endless chain D and carried with it through the ore-chamber, from the entrance to the outlet, returning over the top of the furnace, as shown in the drawings. In passing back over the furnace the chain D and circular plates become sufficiently cooled; the distance travelled by them in the open air being about one hundred feet. With our furnace we do not need to pass the chain through a cooling cistern of water, but, on the contrary, we avoid it, for the reason that the conveyers and hoes, if they entered the furnace wet, would communicate their dampness to the ore, caking it and sticking it to the chain, plate, and hoes so as to interfere with their operation, and accelerate altogether too greatly the forward movement of the ore in the chamber. The furnace is provided with one, two, or three fire-chambers G G, according to the length occupied by the hearth. The first is placed about twenty-five feet from where the ore is fed, and throws the heat about twenty feet, coming in contact with the ore while it is being conveyed from a comparatively cool place and heated up evenly and gradually to 800° Fahrenheit, which heat is increased a little in passing the last fire-chamber.

The operation of our furnace is as follows: The ore is fed in a pulverized state through the hopper H, placed in front of the flue I, and the conveyers are driven slowly by the pulleys. As the conveyers E E', carried along by the chain D, pass slowly through the ore-chamber, the hoes a a a a, projecting down into the ore, plough through its mass, as above described, moving it forward a little every time they pass through it, and thus gradually advancing the whole mass of ore towards the discharge end of the chamber, at the front of the

furnace. As it passes along it is alternately heated and cooled by its position in front of the several fires or in the comparatively cool space between them. This alternate heating and cooling repeated several times is indispensable to the perfect reduction of the ores; for it is not one base metal alone from which we have to free the silver or gold, but many, each of them requiring a different treatment to expel them from the ore, or detach them from the valuable metal which is sought. Once heating and cooling will separate some of the base metals, others will not separate till the ore has been heated to a certain degree—cooled and heated again to a higher degree than before. It is to so alternately heat and cool the mass of ore as to bring to bear upon it successively, during its passage through the furnace, all the conditions required to expel all the base metals usually combined with it, that we have invented our furnace. And we may remark here that in order to perfect the treatment of the ore the several fires should be of different degrees of intensity, preferably increasing their heat as we approach the delivery end of the ore-chamber. The time occupied by these conveyers in passing through the furnace must depend somewhat upon the quality of the ore to be roasted; for a poor or second-class ore the conveyers may be driven rapidly through every six or eight minutes, while the ore is kept stirred at the rate of fifteen or sixteen feet per hour, which gives it about five hours' roasting in an eighty-foot furnace. For ore that requires longer roasting the speed is lessened, and the ore is consequently longer in passing through the furnace. For a longer or shorter furnace the speed is regulated accordingly.

The present way of roasting ores is very imperfect, as well as expensive. The first objection to the Freiberg furnace, and, in fact, all others now in use, is that a portion of the ore lying near the fire-chamber receives too sudden and heavy a heat at first, thereby preventing certain beneficial chemical changes from taking place; and, furthermore, where salt or chlorine is employed, the salt will decompose and the chlorine volatilize before the silver is liberated from the sulphur, and thus leaving the metals to oxidize which will not admit of free amalgamation. The second objection which may be urged in this connection is the stirring in the common furnace. The lighter particles of ore and chlorides will rise and be carried off by the draught; and, thirdly, their arches not being flat enough to confine the heat to the surface and bottom of the ore, the superficial area of the hearth is so great that it becomes necessary to arch the roof in order to secure it, leaving a large space between the roof and surface of the ore; the consequence is much more fuel is required.

By this construction and use of our furnace, we claim to have overcome these imperfections and deficiencies. We heat up gradually and uniformly, the stirring being performed so gently as to lose nothing by draught, confining the heat to the surface and bottom of the ore, and consuming the smoke, our machinery being so perfect that one-horse power and one man will roast the same amount of ore that in other furnaces will require a large power and six men to accomplish the same.

Having thus described our invention, what we claim as new, and desire to secure by Letters Patent, is—

1. The combination and arrangement of the hinged circular plate E E' with the inclined oblique hoes *a a a a*, all constructed as shown, and attached to the endless chain D, substantially as and for the purpose specified.
2. The arrangement of a series of fire-chambers G G along the sides of the ore-chamber of a desulphurizing furnace, at intervals of about twenty-five feet, substantially in the manner and for the purpose set forth.

DAVID J. O'HARRA, [L. S.]  
C. B. THOMPSON. [L. S.]

Witnesses:

A. J. LOCKWOOD,  
JAMES MORRIS.